

## UNITED STATES PATENT OFFICE

KURT SCHMIDT, OF WUPPERTAL-ELBERFELD-GRENZE, GERMANY, ASSIGNOR TO AMERICAN GLANZSTOFF CORPORATION, OF NEW YORK, N. Y., A CORPORATION OF DELAWARE

## FILAMENT TREATMENT

No Drawing. Application filed May 20, 1932, Serial No. 612,658, and in Germany June 8, 1931.

In the manufacture of artificial silk by the well known spool or roller spinning process, the freshly spun filaments are wound directly upon spools. These spools may be 5 either small or large. The artificial silk is then twisted, this being accomplished directly from the smaller spools or after a re-spooling of the larger ones, and brought into the form of skeins. The artificial filaments 10 are then subjected to the different necessary treatments, such as desulphurization, extraction of copper, bleaching, deacidifying, reviving, sizing and dyeing, and are afterwards dried. These steps refer more specifically to artificial filaments produced by 15 the wet spinning process such as from cuprammonium or viscose solutions.

After the development of the process outlined above, it was found that it would be 20 more advantageous to treat the filaments while they were upon the spools rather than while they were in the form of twisted skeins. In order to accomplish this, perforated or foraminous spools were introduced, and the filaments, while upon these 25 spools, were subjected to a treatment by liquids under the influence of either pressure or vacuum. The filaments were then dried and twisted off of the spools to be 30 made up as bottle bobbins, disc spools, cross spools, cones and the like.

A great advantage resides in this process, inasmuch as the time of treatment is shortened considerably. However, a disadvantage 35 has also been found to exist. After the drying of the yarn upon the spools, a product with irregular physical properties resulted because, for the most part, uneven shrinkage of the yarn upon the spools was obtained. The yarn on the inner portion of 40 the spool was subjected to a greater strain than that on the outer portion, and consequently dried unevenly. It was found that even considerable steaming of the yarn did 45 not eliminate these difficulties.

In my new invention, a process is set forth in which the original wet treatment of the 50 yarn in skein form is avoided, but in which unevenness of shrinking is also avoided. My new process may be applied to either the

spool or the roller spinning process, wherein either large or small spools are employed.

The freshly spun artificial yarn is wound upon the spools or rollers in the well known manner and is washed, for example, by the 55 vacuum washing process, and perhaps partially dried during this process. If the large spools, or rollers, are used the yarn is wound upon smaller spools in a known manner in order that it may be twisted. The yarn is 60 then rewound upon secondary supporting devices. These supporting devices are characterized by the fact that they are removable after the completion of the package. They may be in the form of collapsible 65 reels, deformable spools or spools which are provided with a cone taper so that it is possible to draw off the wound package.

One characteristic of the wind upon these 70 secondary supporting means in my present invention, is that the open or honey-combed winding is not necessary, and a very tight comparatively thick winding, in order to produce a cake-like form of the filaments, is used. In order that a cake-like group of 75 filaments may be formed, the spools may be provided with removable flanges or discs in order that well formed edges will be produced.

The next step in my present process is that 80 the packages thus formed are removed from the supporting devices and then subjected to the desired wet treatment and aftertreating processes, such as desulphurization, etc., 85 pointed out above. No reinforcement for the interior of these cakes or packages is necessary.

It has been found advisable in some instances to place cloth or other fabric in the 90 form of a ring shaped cover over the supporting devices prior to the winding processes. This fabric may be of woven or knitted material and is used in order to facilitate the removal of the package from 95 the support. If this protective fabric is long enough it may be also used as a protection for the filaments during their wet treatment. The filaments are thus dried without any support of any sort and therefore 100

the physical irregularities pointed out above are avoided.

I have also found that twine may be laid along the spools prior to the winding thereof and may be used in the manner set forth for the use of the fabric.

The after treatment of these cakes may be performed in many ways, for example, in a pot-shaped perforated vat which varies in size with the size of the package or cake, or by spraying the packages when they are placed on a series of rods. Centrifugal washing may be used either in the vat noted above or by placing the packages upon gridiron-like gratings in large centrifuges, then subjecting them to the treating liquids. They may also be placed upon a support in a series superimposed upon one another, and treated as in the vacuum or pressure washing process. A suitable compression or tightening of the package may be necessary in the event that this latter process is used.

Having now set forth my invention as required by the patent statutes, what I desire to claim is:

1. In a method of treating spun filaments, the steps of spooling the filaments, after-treating with appropriate liquids while on the spool, rewinding and twisting the filaments onto a second supporting means, removing the filaments in the form of a cake from this second support, and further wet treating the said cake.

2. In a method of treating spun filaments, the steps of spooling the filaments, after-treating with appropriate liquids while on the spool, rewinding and twisting the filaments onto a second supporting means, said means being covered with a covering prior to the rewinding of the filaments thereon, removing the filaments in the form of a cake from this second support, and further wet treating the said cake, said covering acting to keep the filaments from tangling or knotting.

3. In a process of the class set forth, the steps of drying spool-spun filaments, rewinding and twisting them onto a second support, removing the filament body so formed, as a unit, and treating this body to aftertreatment and drying while in an unsupported state.

4. In a process of the class set forth, the steps of drying spool-spun filaments, rewinding them onto a second support to form a filament body comprising a tightly wound cake, removing the filament body so formed, as a unit, and treating this body to after-treatment and drying while in an unsupported state.

5. In a process of the type described, the steps of spool spinning and drying filaments, rewinding the yarn into a tight cake onto second supporting means from which the cake may be removed bodily, removing

the cake bodily and then wet treating and drying it while it is in an unsupported condition.

6. In the production of even shrinkage 70 yarn, the steps of spooling spun filaments, respooling onto secondary supports, removing the filaments bodily from said secondary supports, and wet treating and drying them unsupported.

7. In the production of even shrinkage 75 yarn, the steps of spooling spun filaments, wet-treating and drying the yarn while on the spool, respooling onto secondary supports, removing the filaments bodily from 80 said secondary supports, and wet treating and drying them unsupported.

8. In the production of even shrinkage 85 yarn, the steps of spooling spun filaments, respooling onto secondary supports, in the form of a tight cake-like filament body, removing the filaments bodily from 90 said secondary supports, and wet treating and drying them unsupported.

9. In the production of even shrinkage 95 yarn, the steps of spooling spun filaments, wet-treating and drying the yarn while on the spool, respooling onto secondary supports, in the form of a tight cake-like filament body, removing the filaments bodily from 100 said secondary supports, and wet treating and drying them unsupported.

In witness whereof I affix my signature.

KURT SCHMIDT.

100

105

110

115

120

125

130

## DISCLAIMER

1,902,526.—*Kurt Schmidt*, Wuppertal-Elberfeld-Grenze, Germany. FILAMENT TREATMENT. Patent dated March 21, 1933. Disclaimer filed December 6, 1935, by the assignee, *North American Rayon Corporation*.

Hereby enters this disclaimer to those claims numbered 3, 4, 5, 6, and 8, in the said Letters Patent, said claims being in the following words, to wit:

“3. In a process of the class set forth, the steps of drying spool-spun filaments, rewinding and twisting them onto a second support, removing the filament body so formed, as a unit, and treating this body to aftertreatment and drying while in an unsupported state.

“4. In a process of the class set forth, the steps of drying spool-spun filaments, rewinding them onto a second support to form a filament body comprising a tightly wound cake, removing the filament body so formed, as a unit, and treating this body to aftertreatment and drying while in an unsupported state.

“5. In a process of the type described, the steps of spool spinning and drying filaments, rewinding the yarn into a tight cake onto second supporting means from which the cake may be removed bodily, removing the cake bodily and then wet treating and drying it while it is in an unsupported condition.

“6. In the production of even shrinkage yarn, the steps of spooling spun filaments, respooling onto secondary supports, removing the filaments bodily from said secondary supports, and wet treating and drying them unsupported.”

“8. In the production of even shrinkage yarn, the steps of spooling spun filaments, respooling onto secondary supports, in the form of a tight cake-like filament body, removing the filaments bodily from said secondary supports, and wet treating and drying them unsupported.”

[*Official Gazette January 14, 1936.*]